

# UNITED STATES PATENT OFFICE.

GEORG ALEFELD, OF DARMSTADT, GERMANY, ASSIGNOR TO THE PHARMA-ZEUTISCHES INSTITUT LUDWIG WILHELM GANS, OF FRANKFORT-ON-THE-MAIN, GERMANY.

## PROCESS OF PRODUCING INCANDESCENT MATERIALS SUITABLE FOR ELECTRIC LIGHTING.

SPECIFICATION forming part of Letters Patent No. 645,198, dated March 13, 1900.

Application filed February 21, 1899. Serial No. 706,362. (No specimens.)

*To all whom it may concern:*

Be it known that I, GEORG ALEFELD, a citizen of Germany, and a resident of Darmstadt, in the Empire of Germany, have invented a new and useful Improvement in the Production of Incandescent Materials Suitable for Electric Lighting, of which the following is a specification.

Incandescent materials consisting of an inner conductor having an outer covering of metallic oxides are known. Their manufacture, however, is attended with great difficulties. Neither galvanic nor mechanical coatings give satisfactory results, since all attempts to produce an even but sufficiently-thin coating have been unsuccessful. The object of my invention is to overcome these difficulties.

In my process the so-called "lusters" or "lustrous" preparations of the metals are used which have heretofore been sold and used for the decoration of porcelain, glass, &c. These lusters are organic compounds of metals (resin, acid compounds, or sulfureted resin compounds, or products of the decomposition of metallic chlorides produced by heating them with lavender-oil) which are mixed in their application with an ethereal oil, such as lavender-oil. Such lusters of many of the metals are well known, but there is a very remarkable difference between those which have for their basis the so-called "noble" metals—that is, gold, silver, and all the metals of the platinum group—and those which have for their basis the common "unnoble" metals. The first named when applied upon porcelain, glass, or metal and then heated to a high temperature leave behind a thin skin of metal, while the lusters of the unnnoble metals when treated in the same manner form a skin of metallic oxid.

My completed incandescent consists of a core or interior of one of the highly-infusible metals of the platinum group—such as osmium, rhodium, ruthenium, &c., or alloys of the same—covered by an adhesive coherent coating of one of the luminous earthy metals, such as thorium, didymium, cerium, erbium, zirconium, and the like. A mixture of ninety-nine per cent. of thorium and one per cent.

of cerium seems best adapted for this purpose as far as I am at present informed.

I will now describe the two phases of my process, first, the production of the core, and, secondly, the application of the coating to the core.

1. *Production of the core.*—Upon small rods, tubes, or disks of glass or porcelain is spread a solution of a ceramic luster of a highly-infusible metal of the platinum group, such as ruthenium, rhodium, osmium, and the like. Lustrous preparations of these metals may be prepared in an analogous manner to those of gold, silver, and platinum. The small rods, tubes, or disks and the like are coated in straight or curved lines or in any other form with the preparations and then burned in. Mixtures also of these different metals are suitable and form alloys, which are produced in the manner above described. When necessary, the skin of metal thus formed can be strengthened by electrodeposition.

Though known in the art, it may not be amiss to mention that while the lusters of the non-oxidizable noble metals may be burned in without precaution against oxidation the lusters of the oxidizable metals, such as osmium, should be burned in in a reduction-flame, or, better still, in a closed muffle in the presence of a reducing or neutral gas, such as illuminating-gas, hydrogen, or carbonic acid.

The next step is to detach the skin of the noble metal. In order to do that, the glass or the porcelain must be removed, which is done very easily by treating it with hydrofluoric acid or even with hydrochloric acid, provided a special kind of glass soluble in this acid has been used. In so doing it is not at all necessary that the whole of the glass, porcelain, &c., be dissolved before one is able to detach the metal-skin; but generally after a brief treatment with the hydrofluoric acid the metal-skin can be removed as easily as, for instance, a postage-stamp stuck on paper can be removed from the latter by dipping into water; but these skins of the noble metal, particularly if very thin, are easily torn. To avoid such accidents, it is advisable to brush over the skin of noble metal with some form of tough varnish, such as collodion or a gutta-

percha solution, after firing and before endeavoring to detach the skin from the plate. This protecting-coating can be dissolved away by any suitable solvent as soon as the metal-skin is removed from the plate, or it may be allowed to remain indefinitely to protect the metal-skin until its removal becomes desirable.

This hereinbefore-described method of making the core or interior of my incandescent materials being not very convenient for several reasons, a second method has been devised by me which is much better adapted to the purpose. This new process in question has not only been found adapted for producing the core of my incandescents, but serves also for the manufacture of metal foil or leaf, which hitherto could only be obtained by hammering. In an application of even date herewith, Serial No. 706,361, I have explicitly described this method of producing metal foil or leaf. Therefore here I will only repeat the principal points of the process.

A solution of a ceramic luster of an unno-  
ble metal—for example, the resin-acid com-  
pound mixed with an ethereal oil—is spread  
upon the surface of porcelain, glass, metal, or  
any other material which is acid-resistant and  
capable of enduring unimpaired the tempera-  
ture necessary to burn in the ceramic luster  
employed. The luster may be substituted by  
fluxes easily soluble in acid, such as borosili-  
cates or phosphates of soda, &c. Then the  
luster or its substitute is burned in. Upon  
this "bed," as it may be called, a lustrous  
preparation of the desired noble metal is laid  
and burned in in the usual manner. This  
may be repeated until the desired thickness  
is attained, or it may be thickened by elec-  
trolytic deposition of the metal. Then the  
skin of the noble metal is detached by im-  
mersing the plate in a solvent (usually inor-  
ganic and strong organic acids) of the bed,  
which is thus dissolved away, leaving the  
skin of the noble metal free. Before put-  
ting the plate into the solvent the skin  
may be covered with tough varnish, such as  
collodion or a gutta-percha solution, as hereinbefore described. The foil or leaf, still  
covered with the protecting-varnish, if such  
varnish is used, is formed into a thin rod or  
thread by rolling it upon itself or into a tube  
by rolling it around a thread or string or in  
any other suitable manner. The said rod or  
thread or tube is then formed into the de-  
sired shape, and the collodion or varnish and  
the thread or string core, if any, is burned or  
dissolved away. As shown in my said appli-  
cation of even date herewith, Serial No.  
706,361, metal foil or leaf may by its method  
be produced in the form of a sheet or in the  
form of any pattern, so the core of my incan-  
descent body can in accordance with that  
invention be given any desired form—for ex-  
ample, that of a network—by laying the luster  
upon its bed in a reticulated pattern, burn-  
ing it in, and then forming it into a mantle

like those used in gas incandescent lighting, or such a reticulated mantle, or, indeed, almost any form, can be produced by giving the desired form to the porcelain or its substitute, to which the lusters are applied before the first firing.

2. *Applying the coating to the core.*—This core, produced as described, may be used in this form as an incandescent body. In order to strengthen its illuminating power, it may be coated with luminous earthy metal. This second step of my invention is carried out as follows: Upon the core, formed, as hereinbefore described, of one of the highly-infusible metals of the platinum group, is applied a coating of a ceramic resin luster of the desired luminous earthy metal, such as a mixture of ninety-nine per cent. thorium and one per cent. cerium, by dusting it on in the form of a powder or by painting it on or dipping into or otherwise applying a solution or mixture of said resin ceramic luster with an ethereal oil, such as lavender-oil. It is then fired in the usual manner, and the result is an incandescent adapted to incandescent electric lighting, which consists of a core of one of the highly-infusible metals of the platinum group covered with an adherent glass-like coating of a luminous earthy metal. A great practical difference is found in the behavior of these resin compounds of the luminous earthy metals and that of their usual soluble salts—nitrates, acetates, &c.—since with the latter, when fired, the oxid is left behind as a raw powder which has little adhesion, while with the resin compounds a very adherent glass-like coating is produced. My incandescent can then be introduced into an electric circuit in the usual manner and may be used as a substitute for the ordinary carbon filament in a bulb, which in case the core contains one of those metals of the platinum group which are oxidizable in the air, such as osmium, can be evacuated or filled with a reducing or neutral gas, such as illuminating-gas, hydrogen, or carbonic acid. The core is heated by the electric current and heats, in its turn, the exterior coating of the luminous earthy metal to incandescence.

The temperature to which the electric incandescent bodies are heated by the current being far higher than that reached by Auer's incandescent light, even those kinds of earth—for example, lime, magnesia, &c.—can be employed of which the power of light emission is still trifling at the temperature of Auer light, but increases considerably at a higher temperature.

Having thus described my invention, what I claim as new, and desire to patent, is—

1. The within-described process of producing bodies suitable for incandescent electric lighting, which consists: first, in wholly or partially covering a suitable bed with a lustrous preparation of one or more of the highly-infusible metals of the platinum group and burning the same in; second, detaching the

resultant metallic film from the bed by the action of solvents which will attack the bed and not the film; and third, forming the said metallic film into the desired shape.

5 2. The within-described process of producing bodies suitable for incandescent electric lighting, which consists: first, in wholly or partially covering a suitable bed with a lustrous preparation of one or more of the highly-infusible metals of the platinum group and burning the same in; second, covering the metallic film so produced with a tough protective varnish; third, detaching the resultant metallic film from the bed by the action of solvents which will attack the bed and not the film; and fourth, forming the said metallic film into the desired shape.

3. The within-described process of producing bodies suitable for incandescent electric lighting which consists: first, in wholly or partially covering an acid and heat resisting plate or matrix with a ceramic lustrous preparation of one or more of the unnnoble metals and burning the same in; second, laying upon this coating of unnnoble metallic oxid a lustrous preparation of one or more of the highly-infusible metals of the platinum group and burning it in; third, detaching the resultant film of the said highly-infusible metal by the action of a solvent which will attack the unnnoble metallic oxid but not the highly-infusible metal film, and lastly forming the detached film of the highly-infusible metal into the desired shape.

35 4. The within-described process of producing bodies suitable for incandescent electric lighting which consists: first, in wholly or partially covering an acid and heat resisting plate or matrix with a ceramic lustrous preparation of one or more of the unnnoble metals and burning the same in; second, laying upon this coating of unnnoble metallic oxid a lustrous preparation of one or more of the highly-infusible metals of the platinum group and burning it in; third, covering the metallic film so produced with a tough protective varnish; fourth, detaching the resultant film of the said highly-infusible metal by the action of a solvent which will attack the unnnoble metallic oxid but not the highly-infusible metal film, and lastly forming the detached film of the highly-infusible metal into the desired shape.

5. The within-described process of producing bodies suitable for incandescent electric lighting, which consists: first, in wholly or partially covering a suitable bed with a lustrous preparation of one or more of the highly-infusible metals of the platinum group and burning the same in; second, detaching the resultant metallic film from the bed by the action of solvents which will attack the bed and not the film; third, forming the said metallic film into the desired shape; and fourth, coating said so-formed metallic film with ceramic resin luster of one or more of the

luminous earthy metals and burning the same in.

6. The within-described process of producing bodies suitable for incandescent electric lighting, which consists: first, in wholly or partially covering an acid and heat resisting plate or matrix with a ceramic lustrous preparation of one or more of the unnnoble metals and burning the same in; second, laying upon this coating of unnnoble metallic oxid a lustrous preparation of one or more of the highly-infusible metals of the platinum group and burning it in; third, detaching the resultant film of the said highly-infusible metal by the action of a solvent which will attack the unnnoble metallic oxid but not the highly-infusible metal film; fourth, forming the detached film of the highly-infusible metal into the desired shape; and lastly, coating said so-formed metallic film with ceramic resin luster of one or more of the luminous earthy metals and burning the same in.

7. The within-described process of producing bodies suitable for incandescent electric lighting, which consists: first, in wholly or partially covering a suitable bed with a lustrous preparation of one or more of the highly-infusible metals of the platinum group and burning the same in; second, covering the metallic film so produced with a tough protective varnish; third, detaching the resultant film from the bed by the action of solvents which will attack the bed and not the film; fourth, forming the said metallic film into the desired shape; fifth, removing the tough protective varnish from the metallic film by means of a solvent or by burning, using either fire or the electric current, and sixth, coating the metallic film with ceramic resin luster of one or more of the luminous earthy metals and burning the same in.

8. The within-described process of producing bodies suitable for incandescent electric lighting, which consists: first, in wholly or partially covering an acid and heat resisting plate or matrix with a ceramic lustrous preparation of one or more of the unnnoble metals and burning the same in; second, laying upon this coating of unnnoble metallic oxid a lustrous preparation of one or more of the highly-infusible metals of the platinum group and burning it in; third, covering the metallic film so produced with a tough protective varnish; fourth, detaching the resultant film of the said highly-infusible metal by the action of a solvent which will attack the unnnoble metallic oxid but not the highly-infusible metal film; fifth, forming the said metallic film into the desired shape; sixth, removing the tough protective varnish from the metallic film by means of a solvent or by burning, using either fire or the electric current; and seventh, coating the metallic film with ceramic resin luster of one or more of the luminous earthy metals and burning the same in.

9. As a new article of manufacture an incandescent body adapted to incandescent electric lighting, consisting of a core of one or more of the highly-infusible metals of the 5 platinum group, provided with a glass-like coherent and adherent exterior coating of luminous earthy metal as produced by burning in a ceramic resin luster of the same.

Signed at Frankfort-on-the-Main, in the Empire of Germany, this 27th day of January, 10 A. D. 1899.

GEORG ALEFELD.

Witnesses:

RICHARD GUENTHER,  
JEAN GRUND.